# EUROPEAN PATENT SPECIFICATION

(11) **EP 2 158 091 B1**
(45) Date of publication and mention of the grant of the patent: **06.03.2013**
(21) Application number: 08770894.7
(22) Date of filing: 12.06.2008
(51) Int. Cl.: B41M 5/50, C08K 3/08, C09D 5/04

(54) **COATING COMPOSITION**
BESCHICHTUNGSZUSAMMENSETZUNG
COMPOSITION DE REVÊTEMENT

(30) Priority: 15.06.2007 US 764033
(43) Date of publication of application: 03.03.2010
(73) Proprietor: Hewlett-Packard Development Company, L.P., Houston, TX 77070 (US)
(72) Inventor: TOLES, Christopher, San Diego, California 92127-1899 (US); RAYATPARVAR, Mohammed, San Diego, California 92127-1899 (US)
(74) Representative: Beccarelli, Sandra Béatrice Yvonne
(86) International application number: PCT/US2008/066779
(87) International publication number: WO 2008/157261

(56) References cited:
- KR-A- 20010 047 270
- KR-A- 20040 094 796
- KR-A- 20060 085 234
- US-A- 5 405 678
- US-A1- 2005 041 084
- US-A1- 2007 128 349

## Description

### BACKGROUND

Aluminum trihydrate (ATH) is the general name for the chemical compound Al(OH)₃, which occurs as three phases: gibbsite, nordstrandite, and bayerite. Gibbsite is a tabular monclinic crystal with a generally hexagonal outline. Nordstrandite is a triclinic crystal and bayerite is a tabular monoclinic crystal.

Though alumina hydrate, particularly of the boehmite structure, has been used to provide a glossy inkjet media, many grades of aluminum trihydrate particles of sufficiently low costs are too large to function as effective gloss-enhancing layers for inkjet applications. Thus, it would be desirable to provide cost-effective pigment alternatives for paper coating applications, which further provide desirable black optical density and color gamut.

US-A-2007/0128349 discloses a process for preparing an ink-jet recording material which comprises an ink-receptive layer (A) containing fine inorganic particles having an average secondary particle size of 500 nm or less and a resin binder having a keto group on a support.

US-A-2005/0041084 discloses a fast-drying inkjet printable recording media comprising an inkjet printable substrate having multiple coating layers.

### DETAILED DESCRIPTION

In the following description, for purposes of explanation, numerous specific details are set forth in order to provide a thorough understanding of one or more aspects of the disclosure herein. It may be evident, however, that one or more aspects of the disclosure herein may be practiced with a lesser degree of these specific details. The invention is as defined in the claims.

The disclosure relates to an inkjet coating composition and a coated media sheet produced therefrom. The coating composition and coated media sheet have an improved black optical density and high gloss. The coated sheet comprises a substrate, a primary coating layer and a top coating layer. Both single-sided and double-sided coated embodiments are within the scope of the disclosure herein. Here and elsewhere in the specification and claims, the ranges and ratio limits may be combined.

The term "overlies" and cognate terms such as "overlying" and the like, when referring to the relationship of one or a first layer relative to another or a second layer, refers to the fact that the first layer partially or completely overlies the second layer. The first layer overlying the second layer may or may not be in contact with the second layer. For example, one or more additional layers may be positioned between the first layer and the second layer.

In one embodiment, the coating composition is applied to a substrate or media substrate. "Substrate" or "media sheet" includes any material that can be coated in accordance with an embodiment of the disclosure herein, including but not limited to film base substrates, polymeric substrates, conventional paper substrates, clay coated paper, glassine, paperboard, cellulosic paper, photobase substrates, and the like. Further, pre-coated substrates, such as polymeric coated substrates or swellable media, can also be coated in embodiments of the invention.

### Primary Coating Layer

In one embodiment, a "base" or "primary coating" layer overlies the substrate. The primary coating layer may be comprised of a blend of any suitable coating pigments. In one embodiment, the primary coating comprises a blend of an inorganic pigment and a binder. The inorganic pigment may include one or more of alumina, silica, titanium oxide, calcined clay, kaolinite clay, and/or calcium carbonate. In one embodiment, the inorganic pigment comprises calcium carbonate particles. The particulate calcium carbonate is supplied either as mechanically treated natural calcium carbonate material, or as a chemically synthesized reaction product.

The calcium carbonate particles can be ground natural calcium carbonate. Marble, limestone, chalk and coral, for example, are natural sources of calcium carbonate. Alternatively, the calcium carbonate particles can be supplied as a synthetic reaction product in the form of precipitated calcium carbonate. The precipitated calcium carbonate products have a more uniform particle size distribution, and a higher degree of chemical purity, than commercially available ground calcium carbonate.

In addition to the inorganic pigment, the primary coating layer may also comprise a binder. In one embodiment, the primary coating layer contains a binder comprising one or more of polyvinyl alcohol, polyvinyl acetate, polyvinyl acetal, polyacrylic acid and derivatives thereof, starch, cellulosics, carboxycellulosics, polyvinyl pyrrolidone, polyurethane, polyvinyl alcohol (PVA) and derivatives thereof, styrene-butadiene latex, gelatin, alginates, casein, polyethylene glycol (PEG), a poly(vinyl pyrrolidone-vinyl acetate) copolymer, poly(vinyl acetate-ethylene) copolymer, and/or poly(vinyl alcohol-ethylene oxide) copolymer. In one embodiment, the binder comprises PVA. In one embodiment, the binder is present in an amount from about 5 parts (based on 100 parts dry inorganic pigment) to about 50 parts (based on 100 parts dry inorganic pigment). In another embodiment, the binder is present in an amount from about 10 parts (based on 100 parts dry inorganic pigment) to about 25 parts (based on 100 parts dry inorganic pigment).

The primary coating can be applied to the substrate using any coating technique(s), including blade coating, air knife coating, rod coating, gravure coating, cast coating, and/or other techniques, for example. The primary coating layer has a thickness from about 10 to about 35 grams per square meter (g/m²), or from about 15 to about 25 (g/m²) thick. Following application, the primary coating may be dried by any suitable means, such as drum dryers, forced air dryers, gas and/or electric IR dryers, for example.

### Top Coating Layer

In one embodiment, a top coating layer is applied overlying the primary coating layer. The top coating layer comprises an aluminum trihydrate nanopigment and a binder. The ATH nanopigment comprises particulate aluminum trihydrate which has been milled to provide nanoparticles of ATH. The nanoparticles of ATH have a size of less than 180 nanometers (nm). In another embodiment, the ATH nanoparticles are less than 160 nm.

In one embodiment, the ATH nanoparticles account for from about 15wt% to about 40wt% of the milled slurry and in one embodiment, from about 30wt% to about 35wt% of the milled slurry.

The binder for use with respect to the top coating layer can, in one embodiment, comprise one or more binders in common with the binder of the primary coating layer. In one embodiment, the binder of the top coating layer is different than the binder of the primary coating layer. The binder comprises PVA. The PVA comprises a low to medium molecular weight (M_{w}) low percent hydrolysis PVA. In one embodiment, the MW is from about 13,000 to about 30,000, and the percent (%) hydrolysis is from about 86% to about 99%. The amount of binder comprises, in one embodiment, from about 1 part to about 30 parts based upon 100 parts of pigment in the coating. In one embodiment, the amount of binder comprises from about 5 parts to about 20 parts based on 100 parts of pigment in the coating.

In one embodiment the top coating layer comprises a crosslinking agent in an amount from about 0.2 parts to about 5 parts based on 100 parts of pigment in the coating. In one embodiment the top coating layer comprises a crosslinking agent in an amount from about 0.2 parts to about 1 parts based on 100 parts of pigment in the coating. The crosslinking agent comprises one or more of a boron-containing crosslinker, including boric acid, borax, or borates, or a non-boron containing crosslinker, including glyoxal, glutaraldehyde, aldehyde compounds, zirconium sulfate, zirconium acetate, and/or epoxides, for example.

In one embodiment the top coating layer comprises a cationic material. The cationic material may include, for example, one or more of a cationized aluminum chloride-treated silica, pseudoboehmite, cationized kaolinite, aluminum chlorohydrate-treated silica, aminosilane-treated silica, aminosilane-treated kaolinite, and other cationized mineral pigments, and the like. The cationic material is present in an amount from about 15 parts to about 50 parts based on 100 parts of pigment in the coating.

The coating may contain humectants, surfactants, dye fixatives, dyes, optical brighteners, UV absorbers coating rheology modifiers, surfactants, thickeners, deforming agents, preservatives, cast coating releasing agents, fillers, defoamers, lubricants, crosslinkers, dispersants, viscosity modifiers, pH adjusters, defoamers and/or any other suitable additives.

The top coating is prepared by one or more techniques for nanomilling of the ATH particles, including nanomilling, bead milling, horizontal bead milling, planetary ball milling, jet milling (microniser), submicron wet bead milling, and/or colloid milling, for example. A mill is charged with distilled water and sufficient acid to lower the pH to about 2. In one embodiment, an ATH powder is inducted into the mill to bring the total solids up to about 30% to about 40% ATH. The pH is monitored throughout the grind and acid is added to maintain the pH at about 4. Particle size is measured intermittently using light scattering techniques to determine if the particles are in the target size range. When the target size is achieved, the grind is stopped and the dispersion is decanted from the mill. Following formation of the ATH nanopigment, the top coating composition is formed by mixing a slurry of the ATH with binder and water to form an aqueous composition. In one embodiment, the total solids of the top coating composition is about 20 wt%.

The top coating can be applied to the primary coating using any suitable coating device. In accordance with embodiments of the disclosure herein, various coating techniques can be implemented by preparing a coating solution/dispersion to be coated on a media sheet. For example, a substrate can be coated by spray coating, dip coating, cascade coating, swirl coating, extrusion hopper coating, curtain coating, air knife coating, cast coating, rod coating, and/or by using other suitable coating techniques. The thickness selected for each coated layer can depend upon the particular requirement or application and/or by desired properties, as would be ascertainable by one skilled in the art. The top coating is applied, in one embodiment, at a coating weight of about 0.5 g/m² to about 15 g/m². In one embodiment, the top coating is applied at a coating weight of about 10 g/m². The top coating may be applied to at least one surface of the substrate.

Following application of the top coating layer to the substrate, the substrate may be subjected to further processing steps. For example, the substrate may be calendared to further improve gloss or smoothness and other properties of the papers. For example, the substrate is calendared by passing the coated substrate through a nip formed by a calendar roll having a temperature of about room temperature to about 200°C and a pressure of about 689 to about 20684 kPa (kilopascals) (100 to 3000 psi).

### Examples

### Example 1

A primary coating composition was prepared using the Table 1 formulation:

**Table 1**

| **Component** | **Role** | **Dry Parts** |
|---|---|---|
| Calcium carbonate | Inorganic pigment | 60 |
| Calcined kaolinite | Inorganic pigment/spacer | 40 |
| Polyvinyl alcohol | Binder | 0.5 |
| Latex plastic | Binder | 10 |
| Defoamer | Defoamer | 0.2 |
| Surfactant | Wetting agent | 0.2 |

The primary coating was applied to a plain paper sheet substrate at approximately 25 grams per square meter (g/m²) using a meyer rod coating technique. The coated sheet was then dried for approximately 20 to 30 minutes at 120°C in a forced draft oven.

A top coating composition was prepared using the Table 2 formulation:

**Table 2**

| **Component** | **Role** | **Dry Parts** |
|---|---|---|
| Aluminum trihydrate | Inorganic Pigment | 100 |
| Polyvinyl Alcohol | Binder | 10 |
| Boric Acid | Crosslinking Agent | 1 |

The topcoating composition was applied over the primary coating using a #15 Meyer Rod to a coating weight of approximately 10 g/m². The coated sheet was then dried for approximately 20 to 30 minutes at 120°C in a forced draft oven.

The coated sheet was then calendared at a temperature of 93°C and a pressure of 20596kPa (3000psi) for four (4) passes through a calendar (Model 2R-Cal manufactured by Independent Machine, Fairfield, NJ), resulting in a 20° Gloss measurement of 28 and a 60° Gloss measurement of 65, as measured using a Byk-Gardner Tri Gloss Meter.

A print was made using dye ink on an inkjet printer. Black Optical Density was measured using an X-Rite 938 Spectrodensitometer and Color Gamut was measured using a Gretag macBeth Spectroscan unit. The invention coating was compared against a commercial silica-based porous inkjet medium in terms of unprinted gloss, black optical density and color gamut, the results of which are shown in Table 3.

**Table 3**

| **Coating ID** | **Black Optical Density** | **Color Gamut (CieLAB volume)** | **20° Gloss** | **60° Gloss** |
|---|---|---|---|---|
| Silica-based photoglossy inkjet paper | 1.56 | 416,558 | 36 | 57 |
| Example 1 | 1.69 | 386,527 | 28 | 65 |

### Example 2

A top coating composition was made according to the formulations in Table 4:

**Table 4**

| Component | Role | Dry Parts |
|---|---|---|
| Aluminum trihydrate | Inorganic pigment | various |
| Cationic silica | Inorganic pigment | Various |
| Polyvinyl alcohol | Binder | 10 |
| Boric acid | Crosslinking agent | 1 |

The ratio of ATH to cationic silica was varied from 5:1 ATH:silica to 2:1 ATH:silica (dry basis). The topcoats were then applied to the coated base according to Example 1 using a #24 Meyer rod.

The samples were then calendared 2 passes at a temperature of 93°C and a pressure of 20,596kPa (3000psi). 20° and 60° Gloss measurements indicated an unexpected improvement in gloss at an equal ratio of cationized silica:ATH.

### Example 3

A top coating composition was made according to the formulations in Table 5:

**Table 5**

| Component | Role | Dry Parts |
|---|---|---|
| Aluminum trihydrate | Inorganic pigment | various |
| Pseudoboehmite | Inorganic pigment | Various |
| Polyvinyl alcohol | Binder | 10 |
| Boric acid | Crosslinking agent | 1 |

The ratio of ATH to pseudoboehmite was varied from 5:1 ATH:PB to 1:1 ATH:PB (dry basis). The topcoats were then applied to the coated base according to Example 1 using a #24 Meyer rod.

The samples were then calendared 2 passes at a temperature of 93°C and a pressure of 20,596kPa (3000psi). As shown in Table 6, 20° and 60° Gloss measurements indicated an unexpected improvement in gloss at an equal ratio of pseudoboehmite:ATH.

**Table 6**

| **Coating ID** | **20° Gloss** | **60° Gloss** |
|---|---|---|
| ATH Only | 27 | 66 |
| 83% ATH/17% PB | 27 | 63 |
| 50% ATH/50% PB | 27 | 57 |

## Claims

1. A coated media sheet comprising:
a substrate
a primary coating layer;
a top coating layer comprising an aluminum trihydrate nanopigment comprising nanoparticles of less than 180 nm
a binder comprising polyvinyl alcohol (PVA), and
cationized mineral pigment present in an amount ranging from 15 parts to 50 parts based on 100 parts of pigments in the top coating layer

2. The coated media sheet of claim 1, the substrate comprising one or more of film base substrates, polymeric substrates, paper substrates, clay coated paper, glassine, paperboard, cellulosic paper, photodase substrates, pre-coated substrates, polymeric coated substrates and/or swellable media.

3. An inkjet coating composition comprising:
an aluminum trihydrate nanopigment comprising nanoparticles of less than 180 nm a binder comprising polyvinyl alcohol (PVA) in an amount from 1 part to 30 parts per 100 parts of aluminum trithydrate nanopigment and
a cationized mineral pigment present in an amount ranging from 15 parts to 50 parts based on 100 parts of pigments in the too coating layer.

4. The composition of claim 3, comprising a cross-linking agent in an amount from 0.2 parts to 5 parts based on 100 parts of pigment in the composition

5. The composition 4, the cross-linking agent comprising one or more of boric acid, borax, borates, glyoxal, glutaraldehyde, aldehyde compounds, zirconium sulfate, zirconium acetate, and/or epoxides.

6. A method of making a coating composition comprising:
milling a slurry of aluminum trihydrate to form nanoparticles of less than 180 nm thereof;
mixing the slurry of aluminum trihydrate nanoparticles with a binder comprising polyvinyl alcohol, and with a cationized mineral pigment in an amount ranging from 15 parts to 50 parts based on 100 parts of pigments in the top coating layer and with water to form an aqueous coating composition.

7. The method of claim 6, the slurry of aluminum trihydrate comprising from 15wt% to 40wt% aluminum trihydrate.

## Patentansprüche

1. Eine beschichtete Medienbahn, umfassend:
ein Substrat
eine Hauptbeschichtungslage;
eine obere Beschichtungslage, umfassend ein Aluminiumtrihydrat-Nanopigment, umfassend Nanopartikel von weniger als 180 nm ein Bindemittel, umfassend Polyvinylalkohol (PVA) und
ein kationisiertes Mineralpigment, das in einer Menge im Bereich von 15 Teilen bis 50 Teilen basierend auf 100 Teilen an Pigmenten in der oberen Beschichtungslage vorhanden ist

2. Die beschichtete Medienbahn nach Anspruch 1, wobei das Substrat ein oder mehrere Substrate auf Folienbasis, Polymersubstrate, Papiersubstrate, mit Ton beschichtetes Papier, Pergamin, Pappe, Zellulosepapier, Substrate auf Fotobasis, mit Polymer beschichtete Substrate und/oder quellbare Medien umfasst.

3. Tintenstrahl-Beschichtungszusammensetzung, umfassend:
ein Aluminiumtrihydrat-Nanopigment, umfassend Nanopartikel von weniger als 180 nm
ein Bindemittel, umfassend Polyvinylalkohol (PVA) in einer Menge von 1 Teil bis 30 Teilen pro 100 Teilen Aluminiumtrihydrat-Nanopigment und
ein kationisiertes Mineralpigment, das in einer Menge im Bereich von 15 Teilen bis 50 Teilen basierend auf 100 Teilen an Pigmenten in der oberen Beschichtungslage vorhanden ist

4. Zusammensetzung nach Anspruch 3, umfassend ein Vernetzungsmittel in einer Menge von 0,2 Teilen bis 5 Teilen basierend auf 100 Teilen an Pigment in der Zusammensetzung.

5. Zusammensetzung 4, wobei das Vernetzungsmittel ein oder mehrere von Borsäure, Borax, Borate, Glyoxal, Glutaraldehyd, Aldehyd-Verbindungen, Zirkoniumsulfat, Zirkoniumacetat und/oder Epoxiden ist.

6. Verfahren zur Herstellung einer Beschichtungszusammenseztung, umfassend:
das Mahlen eines Schlamms aus Aluminiumtrihydrat zur Bildung von Nanopartikeln von weniger als 180 nm davon;
das Mischen des Schlamms aus Aluminiumtrihydrat-Nanopartikeln mit einem Bindemittel umfassend Polyvinylalkohol und mit einem kationisierten Mineralpigment in einer Menge im Bereich von 15 Teilen bis 50 Teilen basierend auf 100 Teilen an Pigmenten in der oberen Beschichtungslage sowie mit Wasser zum Bilden einer wässrigen Beschichtungszusammensetzung.

7. Verfahren nach Anspruch 6, wobei der Schlamm aus Aluminiumtrihydrat von 15 Gew.-% bis 40 Gew.-% an Aluminiumtrihydrat umfasst.

## Revendications

1. Feuille de support revêtue comprenant :
- un substrat ;
- une couche de revêtement primaire ;
- une couche de revêtement supérieure comprenant un nanopigment de trihydrate d'aluminium comprenant des nanoparticules de moins de 180 nm ;
- un liant comprenant de l'alcool polyvinylique (PVA) ; et
- un pigment minéral cationisé présent dans une quantité se situant dans une plage de 15 parties à 50 parties sur la base de 100 parties de pigments dans la couche de revêtement supérieure.

2. Feuille de support revêtue selon la revendication 1, le substrat comprenant un ou plusieurs parmi les substrats de base de film, les substrats polymères, les substrats de papier, le papier couché au kaolin, le papier cristal, le carton, le papier cellulosique, les substrats de photobase, les substrats pré-revêtus, les substrats revêtus par un polymère et/ou les supports gonflables.

3. Composition de revêtement pour jet d'encre comprenant :
- un nanopigment de trihydrate d'aluminium comprenant des nanoparticules de moins de 180 nm ;
- un liant comprenant l'alcool polyvinylique (PVA) dans une quantité de 1 partie à 30 parties pour 100 parties de nanopigment de trihydrate d'aluminium ; et
- un pigment minéral cationisé présent dans une quantité se situant dans une plage de 15 parties à 50 parties sur la base de 100 parties de pigments dans la couche de revêtement supérieure.

4. Composition selon la revendication 3, comprenant un agent réticulant dans une quantité de 0,2 partie à 5 parties sur la base de 100 parties de pigment dans la composition.

5. Composition selon la revendication 4, l'agent réticulant comprenant un ou plusieurs parmi l'acide borique, le borax, les borates, le glyoxal, le glutaraldéhyde, les composés aldéhydes, le sulfate de zirconium, l'acétate de zirconium et/ou les époxydes.

6. Procédé de fabrication d'une composition de revêtement, comprenant les opérations consistant à :
- mélanger une bouillie de trihydrate d'aluminium pour former des nanoparticules de moins de 180 nm de celui-ci ;
- mélanger la bouillie de nanoparticules de trihydrate d'aluminium avec un liant comprenant de l'alcool polyvinylique et avec un pigment minéral cationisé dans une quantité se situant dans une plage de 15 parties à 50 parties sur la base de 100 parties de pigments dans la couche de revêtement supérieure et avec de l'eau pour former une composition aqueuse de revêtement.

7. Procédé selon la revendication 6, la bouillie de trihydrate d'aluminium comprenant de 15 % en poids à 40 % en poids de trihydrate d'aluminium.
